

3,230,078

## MANGANESE-BASE ALLOYS

Alfred William Owen Webb and Norman Bailey, Kent, England, assignors to J. Stone & Company (Propellers) Limited, London, England, a company of Great Britain  
No Drawing. Filed Jan. 7, 1963, Ser. No. 249,578  
4 Claims. (Cl. 75—134)

This invention concerns improvements relating to manganese-base alloys. Manganese-copper alloys containing between about 10 and 55% of copper have high damping capacity and a variety of alloys have been developed, based on this binary system, which have useful properties for particular applications.

The possession of a high damping capacity is very desirable in an alloy for marine propellers, but for this purpose the said capacity must be accompanied by sufficiently high strength, fatigue resistance, erosion resistance and corrosion resistance. Also, it must be capable of being melted and cast by the conventional methods by which very large propeller castings are produced. Alloys which have been produced heretofore do not possess all these characteristics together. In general, they are difficult to cast and have inferior mechanical properties in the cast condition.

A series of alloys based on the manganese-copper system and containing aluminium and nickel has now been developed, in which the damping capacity in the cast condition is better than that of the binary alloys, and in which high damping capacity can be obtained without the need for heat-treatment. These new alloys also have reason-

added up to 2.5% without significant change in the cast structure, although the damping capacity falls to some extent. When more than 2.5% of aluminium is added, however, two new phases appear; namely a body-centred cubic phase similar to the beta phase in aluminium bronzes, and a phase believed to be a complex ternary compound  $Cu_3Mn_2Al$ . When the body-centred cubic phase appears in small amounts, the damping capacity of the alloy increases significantly, while the tensile properties and machineability of the alloy are also improved. The amounts of both of the new phases increase as the aluminium content is raised, but above 6% of aluminium the damping capacity falls once more and the tensile properties of the alloy also deteriorate. Thus alloys containing between 2.5% and 6% of aluminium have exceptionally good damping capacity and tensile properties, and are easier to machine than alloys outside these limits of composition. The presence of aluminium in these amounts also improves the casting characteristics. The addition of nickel further improves the tensile properties and in conjunction with aluminium also improves the resistance to corrosion. The addition of nickel has no significant effect on the amounts of the aforesaid body-centred cubic phase and complex ternary compound when added in amounts up to 5%, but it appears to have an influence on the precipitation of alpha-manganese and, if the nickel content exceeds 3.5%, the damping capacity begins to fall rapidly, although below this level nickel appears to have a slightly beneficial effect on damping capacity. The effects of variations in nickel content upon the tensile properties and damping capacity are indicated in Table I.

Table I

| Chemical Composition, Percent |        |                |        |      |         |        | 0.1% Proof Stress, tons/in. <sup>2</sup> | Tensile Strength, tons/in. <sup>2</sup> | Elongation, Percent | Youngs Modulus, lb./in. <sup>2</sup> X10 <sup>-3</sup> | Specific Damping Capacity, Percent |
|-------------------------------|--------|----------------|--------|------|---------|--------|------------------------------------------|-----------------------------------------|---------------------|--------------------------------------------------------|------------------------------------|
| Manganese                     | Copper | Alum-<br>inium | Nickel | Iron | Silicon | Carbon |                                          |                                         |                     |                                                        |                                    |
| 51.0                          | 40.9   | 4.4            | 0.5    | 2.7  | 0.05    | 0.12   | 18.3                                     | 37.2                                    | 26                  | 12.0                                                   | 19.5                               |
| 52.6                          | 38.1   | 4.5            | 1.5    | 3.1  | 0.07    | 0.12   | 17.4                                     | 37.1                                    | 34                  | 11.0                                                   | 28                                 |
| 53.7                          | 35.2   | 4.8            | 3.5    | 2.7  | 0.08    | 0.02   | 18.2                                     | 41.4                                    | 34                  | 13.0                                                   | 9.5                                |
| 53.2                          | 34.8   | 4.7            | 4.3    | 2.7  | 0.09    | 0.02   | 18.2                                     | 41.5                                    | 36                  | 15.3                                                   | 4                                  |

able casting characteristics and good mechanical properties.

An alloy in accordance with the present invention contains 25 to 50% of copper, 2.5 to 6% of aluminium and 0.5 to 3.5% of nickel, the rest (except for impurities and incidental constituents) being manganese, which amounts to at least 47%, carbon or silicon present amounting to less than 0.2% respectively. Preferably the manganese content does not exceed 60% and the copper content does not exceed 48%. Iron may be present in amounts up to 5% and tin in amounts up to 2%.

Alloys with such a composition not only possess a high damping capacity and good tensile strength, but may also have a corrosion fatigue resistance greater than that of high tensile brass, which has long been used for marine propellers. For instance, an alloy containing 54.6% of manganese, 36.0% copper, 4.5% of aluminium, 2.1% of nickel, 2.9% of iron, 0.06% of silicon and 0.04% of carbon had an endurance limit in salt spray, based on 10<sup>8</sup> reversals of stress, of  $\pm 7.75$  tons/in.<sup>2</sup>, which compares favourably with values of about  $\pm 6$  tons/in.<sup>2</sup> for accepted propeller alloys.

Binary manganese-copper alloys consist of a matrix of face-centred cubic solid solution containing precipitated particles of alpha-manganese. Aluminium may be

50 The damping capacity values in Table I may be compared with specific damping capacities of 0.3% for a typical high tensile brass, and 10.6% for a cast iron containing about 3.5% of carbon, the latter value being regarded as a good damping capacity.

55 The damping capacity increases with manganese content up to a maximum at about 70% manganese. On the other hand, tensile properties deteriorate at manganese contents about 60%, and the casting characteristics are also better with alloys of lower manganese content. For instance, the liquidus temperature decreases with decrease in manganese content, the liquidus points of alloys with 70 and 47% of manganese being 1150 and 990° C. respectively, so that it is easier to maintain freedom from oxide inclusions and gas in the case of alloys with lower manganese content. The width of the freezing range is also reduced as the manganese content is lowered, and 60 this reduces the liability of the alloys to shrinkage porosity. Because of this, the most generally useful alloys are likely to have manganese contents close to but slightly below 60%.

65 The damping capacity is critically dependent upon the silicon and carbon contents, again because they appear to interfere with the form of precipitation of alpha-manganese. If either the silicon content or the carbon content

exceeds 0.2%, the damping capacity of the alloy becomes very low, as shown by the following table:

The alloys are also capable of being hot worked by forging and other processes. Such processes can impair

Table II

| Chemical Composition, Percent |        |                |        |      |         |        | 0.1%<br>Proof<br>Stress,<br>tons/in. <sup>2</sup> | Tensile<br>Strength,<br>tons/in. <sup>2</sup> | Elonga-<br>tion,<br>Percent | Youngs<br>Modulus,<br>lb./in. <sup>2</sup><br>X10 <sup>-6</sup> | Specific<br>Damping<br>Capacity,<br>Percent |
|-------------------------------|--------|----------------|--------|------|---------|--------|---------------------------------------------------|-----------------------------------------------|-----------------------------|-----------------------------------------------------------------|---------------------------------------------|
| Manganese                     | Copper | Alu-<br>minium | Nickel | Iron | Silicon | Carbon |                                                   |                                               |                             |                                                                 |                                             |
| 52.6                          | 37.6   | 4.3            | 1.5    | 3.2  | 0.09    | 0.10   | 17.9                                              | 37.4                                          | 31                          | 10.5                                                            | 26.5                                        |
| 52.4                          | 37.4   | 5.0            | 1.6    | 3.2  | 0.19    | 0.38   | 22.4                                              | 38.8                                          | 8                           | 14.7                                                            | 3.5                                         |
| 54.6                          | 36.1   | 4.5            | 2.1    | 2.9  | 0.06    | 0.04   | 17.6                                              | 37.7                                          | 33                          | 11.8                                                            | 20                                          |
| 55.0                          | 34.4   | 4.8            | 2.0    | 2.9  | 0.28    | 0.61   | 27.0                                              | 36.9                                          | 0.5                         | 16.1                                                            | 4                                           |

Contents of the elements silicon and carbon must, therefore, never exceed the said limits. Amounts of these elements in excess of the said limits also harden and embrittle the alloy and impair its machineability. They also increase the freezing range, thereby impairing the castability, particularly with alloys having a high manganese content.

Small additions of tin improve the resistance to corrosion, but in amounts exceeding 2%, tin embrittles the alloy. The presence of iron has relatively little effect on the damping capacity or tensile properties, but is advantageous in improving the resistance to impingement corrosion. Its addition is therefore beneficial, except in alloys containing tin, where it should be kept to a very low level.

Other elements may be added for specific known purposes, for example lead in amounts up to 1% may be added to ensure a free-machining alloy without impairing either damping capacity or mechanical properties.

Typical tensile properties and damping capacities for alloys in accordance with the invention are given by the following table:

15 the damping capacity, but the alloys are susceptible to heat-treatment, which can be used to restore this capacity. The improved casting characteristics of the alloys described allow the manufacture of sound billets and ingots for further working.

20 This invention comprises also propellers and propeller castings made from alloys having the composition hereinbefore set forth.

We claim:

25 1. A casting having high damping capacity constituted of an alloy consisting essentially of from 25 to 50% of copper, 2.5 to 6% of aluminium, and 0.5 to 3.5% nickel, the rest being essentially manganese, in an amount of at least 47%, and any carbon and silicon present, as impurities, amounting to less than 0.2%, respectively.

2. A casting as claimed in claim 1, wherein the alloy contains iron in an amount up to 5%.

3. A casting as claimed in claim 1, wherein the alloy contains tin in an amount up to 2%.

4. A casting as claimed in claim 1, wherein the alloy contains lead in an amount up to 1%.

Table III

| Chemical Composition, Percent |        |                |        |      |       |       |         |        | 0.1%<br>Proof<br>Stress,<br>tons/in. <sup>2</sup> | Tensile<br>Strength,<br>tons/in. <sup>2</sup> | Elonga-<br>tion,<br>Percent | Youngs<br>Modulus,<br>lb./in. <sup>2</sup><br>X10 <sup>-6</sup> | Specific<br>Damping<br>Capacity,<br>Percent |
|-------------------------------|--------|----------------|--------|------|-------|-------|---------|--------|---------------------------------------------------|-----------------------------------------------|-----------------------------|-----------------------------------------------------------------|---------------------------------------------|
| Manganese                     | Copper | Alu-<br>minium | Nickel | Iron | Tin   | Lead  | Silicon | Carbon |                                                   |                                               |                             |                                                                 |                                             |
| 52.0                          | 38.2   | 4.6            | 2.1    | 3.1  | ----- | ----- | 0.02    | 0.02   | 18.5                                              | 40.2                                          | 30                          | 13.2                                                            | 15                                          |
| 52.6                          | 38.1   | 4.5            | 1.5    | 3.1  | ----- | ----- | 0.07    | 0.12   | 17.4                                              | 37.1                                          | 34                          | 11.0                                                            | 28                                          |
| 59.8                          | 30.7   | 4.6            | 2.0    | 2.9  | ----- | ----- | 0.02    | 0.08   | 17.5                                              | 39.1                                          | 30                          | 10.9                                                            | 24                                          |
| 49.6                          | 44.4   | 3.8            | 1.5    | 0.07 | 0.40  | ----- | 0.02    | 0.03   | 17.0                                              | 37.4                                          | 35                          | 11.3                                                            | 19                                          |
| 56.0                          | 37.0   | 4.8            | 2.0    | 0.06 | ----- | ----- | 0.06    | 0.14   | 19.0                                              | 40.6                                          | 20                          | 10.8                                                            | 21                                          |
| 51.3                          | 42.1   | 4.9            | 1.6    | 0.06 | ----- | ----- | 0.01    | 0.06   | 17.8                                              | 40.6                                          | 30                          | 11.7                                                            | 22                                          |
| 50.7                          | 39.9   | 4.1            | 1.4    | 3.2  | ----- | 0.18  | 0.02    | 0.07   | 17.1                                              | 35.8                                          | 33                          | 11.2                                                            | 21                                          |
| 65.4                          | 25.0   | 4.8            | 2.1    | 2.6  | ----- | ----- | 0.03    | 0.01   | 14.4                                              | 34.8                                          | 42                          | 8.8                                                             | 30                                          |

With such alloys, a high damping capacity can be obtained in the cast condition provided that cooling rates through the temperature range 500-300° C. are not excessively fast, i.e. are not such as may occur in the case of die castings or other thin walled castings. If necessary, however, the damping capacity of such fast-cooled castings can be improved by heat-treatment within the temperature range 500-300° C.

## References Cited by the Examiner

## UNITED STATES PATENTS

55 2,287,888 6/1942 Kroll ----- 75-134.9 X  
2,310,094 2/1943 Kroll ----- 75-134.9 X

HYLAND BIZOT, Primary Examiner.

DAVID L. RECK, Examiner.